

Patented Oct. 17, 1944

2,360,631

# UNITED STATES PATENT OFFICE

2,360,631

## LUBRICANT

John C. Zimmer, Union, and Arnold J. Morway,  
Clark Township, Union County, N. J., assign-  
ors to Standard Oil Development Company, a  
corporation of Delaware

No Drawing. Application December 9, 1942,  
Serial No. 468,422

8 Claims. (Cl. 252—36)

The present invention relates to improved stable lubricating compositions, particularly to lubricating greases stable at high temperatures. More particularly the invention relates to grease compositions suitable for the lubrication of sealed anti-friction bearings, such as ball bearings and roller bearings.

It is known in the art to prepare various lubricating grease compositions adapted for particular uses. The uses in which grease compositions are employed present a wide variety of conditions and generally a grease prepared with a given set of conditions in mind is not suitable for use under a different set of conditions. The operation of mechanical mechanisms either at high temperatures or in the proximity of high temperatures offers a difficult lubrication problem particularly where greases are used as the lubricant. Although not unique in this respect, small electrical generators, such as those attached to internal combustion engines provide a convenient example of the requirements in high temperature lubrication. In their construction these generators contain sealed and lubricated anti-friction bearings which it is contemplated will not need replacement during the life of the generator. When the motors to which these generators are attached are operated over an extended period of time, these generators due to heat radiation, conduction and other causes, attain temperatures which ordinary greases will not withstand.

High temperature greases such as the sodium soap greases containing excess alkali are known to the art. However, they are quite water-soluble and readily disintegrate under humid conditions and unless properly made are not stable in storage. This instability in storage is evidenced by separation occurring between the oil and the soap. To overcome this instability in storage, large amounts of high molecular weight sodium soaps, say 25% or more, have been used in compounding the grease. Although the conventional greases containing these large amounts of soap do not bleed oil in storage they possess operational defects in that at temperatures above 200° F. they become stiff and hard, readily oxidize and lose the soft consistency desired in greases particularly when prepared from low viscosity oils, i. e. below 100 secs. at 210° F.

The principal object of the present invention is to produce a grease composition which will provide adequate lubrication at both high and low temperatures and one that will not at high temperatures increase the running torque of the mechanism lubricated. Another object is to pro-

vide a high temperature grease which is stable against bleeding during storage. Other and further objects will be apparent to those skilled in the art from a reading of the following description.

5 The grease composition made in accordance with the present invention comprises essentially a low pour point lubricating mineral oil distillate, an alkali soap of an unsaturated fatty acid and a saturated fatty acid soap of an amphoteric metal. It has now been found that it requires less of the soaps of the fatty acids obtained from rape seed oil or mustard seed oil which contain high percentages of erucic acid, to produce a grease 10 which is stable in storage. Greases containing soaps of these acids, particularly those soaps having some excess alkali which is necessary to preserve the high heat resistance, do not possess desirable resistance to the action of water. It has 15 further been discovered that by the use of small amounts of saturated fatty acid soaps of amphoteric metals, the compositions of the invention can be made to appear neutral or slightly acid to a hydrogen ion indicator such as phenol-phthalein, thus attaining the water-resistance of a 20 neutral or acid grease while preserving the high heat resistivity of the slightly alkaline greases. The greases of the present invention are especially advantageous in that stability during storage is obtained without at the same time producing a grease which becomes stiff and hard 25 at temperatures above 200° F. The greases of the present invention do not lose their grease consistency or become thick and stiff at temperatures as high as 400° F. A small amount of an 30 anti-oxidant such as say 0.2% of phenyl alpha naphthylamine, dyes or other addition agents may be added if desired, for example metal deactivators, extreme pressure agents, etc.

40 Although any of the numerous types of low pour point lubricating oils may be used as the base for compositions made nearly in accordance with this invention, it is preferred to use a Coastal type oil having a viscosity in the range of from about 50 to 1000 seconds S. U. V. at 100° F. and a cold test below 0° F.

45 For the formation of the soaps utilized in the production of the greases any fat or fatty acid, such as mustard oil or rapeseed oil, containing erucic acid, which is an unsaturated acid of 22 carbon atoms to the molecule, may be used. For the production of the soaps of the amphoteric metals it is preferred to use stearic acid, although any of the other well-known saturated acids of high molecular weight such as the

saturated acids derived from hydrogenated fish oil may be used. The amphoteric metals which are well established and recognized in the art are amply illustrated by zinc, aluminum, or iron. Instead of employing saturated fatty acid soaps of amphoteric metals, the naphthenates, or salts of any acid having an iodine number under 30 combined with amphoteric metals will be found to function with equal facility.

Any of the methods customarily employed in the compounding of greases may be used in the production of the compositions of this invention. The soaps may be produced separately and then mixed with the oil by heat and agitation or preferably the fat or fatty acids to be combined with the alkali may be dissolved in a portion of the lubricating oil by heating the oil sufficiently to dissolve the fat or acid in the oil, reacting the fat or fatty acid with sodium hydroxide, or other alkali metal hydroxide such as lithium hydroxide, or alkaline earth metal hydroxide, such as calcium hydroxide, preferably dissolved in water, and then the remainder of the lubricating oil having the soap of the amphoteric metal dispersed therein may be added after which the mixture is brought to a clear solution and the water driven off by heating and stirring, the anti-oxidant added and the mixture permitted to cool. It is preferred to make the soap of the amphoteric metal separately and then dissolve it in a portion of the lubricating oil although it is quite possible to produce the soap of the amphoteric metal in situ in the oil. Greases of varying consistency to meet the demands of particular conditions may be secured by varying the soap content of the grease within specified limits. The composition of the grease will be approximately as follows: The quantity of oil in the grease will range from about 74% to 89.75%, alkali soaps of fatty acids in which erucic acid predominates will range from about 10% to 25% and the soap of amphoteric metal will run from about 0.25% to 1% with varying amounts up to 0.5% of other additives such as oxidation inhibitors. The following examples will serve to illustrate specific embodiments of the invention.

*Example I*

|                                        | Per cent |
|----------------------------------------|----------|
| Rapeseed oil                           | 20.0     |
| Aluminum stearate                      | 1.0      |
| NaOH                                   | 3.0      |
| Lubricating oil (low pour Coastal oil) | 76.4     |

20 parts by weight of the rapeseed oil were mixed with 25 parts of the hydrocarbon lubricating oils. This mixture was then heated while stirring until about 150° F., whereupon a 25% solution of caustic soda was added, the amount being about 3% of dry caustic soda. Heat was continued until all water was driven off (an analysis of the grease at this stage should show a free alkalinity of approximately 0.05 to 0.15% as NaOH). The aluminum stearate dispersed in a small amount of the oil together with the balance of the oil was then added. The temperature was then raised to 400/450° F. at which temperature heating was discontinued. The grease was stirred until the temperature had dropped to 180° F. and then drawn off. The grease thus produced tested as follows:

|                    |         |
|--------------------|---------|
| Penetration        | 192     |
| Worked penetration | 195     |
| Melting point      | °F. 400 |

Several drops of a .05% solution of phenolphthalein placed on a film of the grease at room temperature showed no change of color after 15 minutes.

5

*Example II*

Per cent

Fatty acids obtained from mustard oil or containing substantial amounts of erucic acid

|                                        |       |
|----------------------------------------|-------|
| 10                                     | 13.00 |
| Zinc naphthenate                       | 0.50  |
| Aluminum stearate                      | 0.50  |
| NaOH                                   | 1.67  |
| Lubricating oil (low pour Coastal oil) | 82.83 |

15

This grease prepared by the method described in Example I showed the following characteristics:

|                    |         |
|--------------------|---------|
| Penetration        | 276     |
| Worked penetration | 280     |
| Melting point      | °F. 370 |

No effect on phenolphthalein solution.

What is claimed is:

1. An improved lubricating grease composition comprising a low pour point lubricating mineral oil distillate, 10-25% of an alkali soap containing excess alkali, a substantial portion of which is a soap of a mono carboxylic, mono olefinic aliphatic acid of twenty-two carbon atoms and 30 0.25-1% of a soap of an amphoteric metal and an acid having an iodine number under 30.

2. A composition as defined by claim 1 in which the soap of an amphoteric metal and an acid having an iodine number under 30 is aluminum stearate.

3. A composition as defined by claim 1 in which the soap of an amphoteric metal and an acid having an iodine number under 30 is zinc naphthenate.

4. An improved lubricating grease composition comprising a low pour point lubricating mineral oil distillate, 10-25% of the sodium soap of a mono carboxylic, mono olefinic aliphatic acid of 22 carbon atoms containing excess soda and 45 0.25-1% of a plurality of soaps of amphoteric metals and acids having an iodine number under 30.

5. An improved lubricating grease composition comprising a low pour point lubricating mineral oil distillate, 10-25% of the sodium soap of erucic acid containing excess soda and from 0.25-1.0% aluminum stearate.

6. An improved lubricating grease composition comprising a low pour point lubricating mineral oil distillate, 10-25% of the sodium soap of erucic acid containing .05-.15% excess soda, 0.5% aluminum stearate and 0.5% zinc naphthenate.

7. An improved lubricating grease composition comprising a low pour point lubricating mineral oil distillate, 10-25% of the sodium soap of mono carboxylic acids derived from rape seed oil containing .05-.15% excess soda and .25-1% of a plurality of soaps of amphoteric metals and acids having an iodine number under 30.

8. An improved lubricating grease composition comprising a low pour point lubricating mineral oil distillate, 10-25% of the sodium soap of mono carboxylic acids derived from mustard seed oil 70 containing .05-.15% excess soda, 0.5% aluminum stearate and 0.5% zinc naphthenate.

JOHN C. ZIMMER.  
ARNOLD J. MORWAY.